

# UNITED STATES PATENT OFFICE.

WILLEM TOM, OF KATWIJK AAN ZEE, NETHERLANDS.

## COMPOSITION FOR IMPREGNATING FIBROUS MATERIALS.

No Drawing. Application filed November 1, 1926, Serial No. 145,696, and in the Netherlands October 28, 1925.

This invention relates to the treatment of fibrous materials, such as cotton, hemp and the like, and of articles made from such materials.

For certain purposes, e. g., in the equipment of ships, and particularly for ropes, it has heretofore been found necessary to utilize manila hemp, which material, when treated with tar, is able to withstand the influences of weather and of sea water.

The invention renders possible the substitution for manila hemp of fibrous materials which have heretofore been considered unsuitable because insusceptible to treatment to adapt them to answer requirements.

The invention is based on the discovery of a product suitable for the impregnation of such fibrous materials and of articles composed of such materials which endows them with the required properties.

Essentially, the product in question is compounded of paraffin, petroleum jelly, naphthaline and turpentine in intimate admixture.

For the preparation of this product a mixture of molten paraffin solid at normal temperatures and petroleum jelly is first heated to a temperature between 70° and 80° C., to form a homogeneous mass which is then fur-

ther heated to a temperature between 100° and 130° C., preferably 120° to 130° C., whereupon naphthaline is added. The mix-

ture of paraffin, petroleum jelly and naphthaline is then allowed to cool to a temperature between 90° and 80° C., at which point turpentine is added, preferably while stirring. The mixture in warm condition is available for the immediate impregnation of the fibrous materials or it may be allowed to

solidify and be stored in barrels, it being understood that in this event it requires to be reheated for use as an impregnating agent.

Suitable proportions for the ingredients are as follows, the measurements being by weight:—15 to 30% paraffin, 6 to 15% petroleum jelly, and 3 to 10% naphthaline, the remainder being turpentine.

The fibrous materials or articles prepared from such materials are impregnated with the mixture aforesaid, the latter being at a temperature of about 80° C., and then dried centrifugally or otherwise and exposed to the air.

It is found that fibrous materials so impregnated, without any other treatment, are capable of withstanding the influence of water, especially of sea water, and have a long life. This is particularly true of hemp fibres, particularly from Java, which are naturally unsuited to withstand the influence of sea water.

In lieu of treating the materials in fibrous form I may treat finished articles prepared from fibrous materials, such, for example, as fishing nets.

By "petroleum jelly" is meant the commodity sold as vaseline.

I claim:—

A composition for impregnation of fibrous materials or articles made from fibrous materials consisting of a homogeneous mixture of 15 to 30% of paraffin, 6 to 15% petroleum jelly, 3 to 10% naphthalene, and turpentine.

In testimony whereof I have signed my name to this specification.

W. TOM.